# EUROPEAN PATENT SPECIFICATION

(11) **EP 0 218 167 B1**
(45) Date of publication and mention of the grant of the patent: **28.11.1990**
(21) Application number: 86113353.6
(22) Date of filing: 29.09.1986
(51) Int. Cl.: C21D 7/04, C21D 8/06, C22C 38/04

(54) **High tensile strength drawn steel wire with improved ductility**
Gezogener Stahldraht mit hoher Bruchfestigkeit und Duktilität
Fil d'acier tréfilé à haute résistance à la rupture et à ductilité modifiée

(30) Priority: 30.09.1985 JP 214770/85; 30.09.1985 JP 214771/85; 30.09.1985 JP 214977/85
(43) Date of publication of application: 15.04.1987
(73) Proprietor: NIPPON STEEL CORPORATION, Tokyo 100 (JP)
(72) Inventor: Takahashi, Toshihiko Dainigijutsukenkyusho, Sagamihara-shi (JP); Asano, Yoshiuki Dainigijutsukenkyusho, Sagamihara-shi (JP)
(74) Representative: VOSSIUS & PARTNER

(56) References cited:
- DE-C- 747 761
- FR-A- 678 070
- GB-A- 531 017
- GB-A- 712 125
- PATENTS ABSTRACTS OF JAPAN, vol. 7, no. 61 (C-156)[1206], 15th March 1983; & JP-A-57 210 916 (SUMITOMO DENKI KOGYO K.K.) 24-12-1982
- STAHL UND EISEN, vol. 104, no. 14, 9th July 1984, pages 657-660, Düsseldorf, DE; E. von FINCKENSTEIN et al.: "Eigenspannungen beim Oberflächen-Feinwalzen"
- WIRE JOURNAL INTERNATIONAL, vol. 16, no. 4, 1983, pages 50-61, Guildford, US; K. AIHARA et al.: "High-strength and high-fatigue limit zinc galvanized steel cord for ACSR"
- Herstellung von Stahldraht , Teil 1 ,pages 187,225,257-260, Verein Deutscher Eisenhüttenleute , 1969

## Description

The present invention relates to a high tensile strength drawn steel wire having excellent ductility, and to a method of producing such a steel wire.

In hard drawn steel wires which are used as steel wire for ropes, as tire reinforcing steel wire, as optical fiber cable reinforcing steel wire or as steel wire for suspension bridges, it is increasingly needed to strengthen the wires.

Studies to increase the strength of hard drawn steel wires have been conducted energetically, but their strength has not yet reached an adequate level. This is caused by the fact that increases in strength deteriorate the ductility, and the technology for prevention of this deterioration has not yet been established. The torsional characteristics of steel wires, which are regarded as the criteria for ductility, can be improved by bluing drawn steel wires at a high temperature, as described on page 50 of Wire Journal Vol. 16, No. 4 (1983). Such a high temperature processing, however, leads to a decrease in the strength of the wire. In addition, it oxidizes the surface of small-gage wires used as tire reinforcing steel wires and thereby diminishes their ductility. Thus, its application has been limited.

Apart from this heat processing, an attempt has been made to increase ductility by releasing the residual tensile stress present on the surface of a drawn steel wire by skin pass drawing of the drawn steel wire. However, this process is not capable of improving the ductility, as described in a paper with the title "Effect of Dies Schedule on Mechanical Properties and Residual Stress of Steel Wire" which was submitted to the Drawing Technology Subcommittee of the Japan Society for Plastic Processing.

It has been known to impart residual compression stress to the surface of a steel wire for the purpose of increasing fatigue properties. However, there is no apparent relationship between the fatigue properties and ductility, as is described on page 392 of "Strength and Fracture of Iron and Steel Materials (1964)". This means that it is not possible to derive a method to improve the ductility from a method of improving the fatigue properties.

Thus, known methods of increasing ductility of steel wires have all proved inadequate.

In "Wire Journal International" Vol. 16, No. 4, 1983, page 50 to 61, the development of a new zinc galvanized steel cord for ACSR (aluminum conductor steel reinforced) having high strength and high fatigue limit is discussed. The steel comprises 0.81% C, 0.89% Si, 0.44% Mn, 0.019% P, 0.010% S, 0.33% Cr, 0.001% sol. AI and 0.004% N, the above composition referring to % by weight. The development discussed in this article aims at attaining a tensile strength of more than 180 kgf/mm² in the finished wire but the article does not discuss any improvement of the ductility of said wire by the application of a residual compression stress on the surface of the wire.

Various attempts are known to improve various steel properties, like the durability, the strength of the wire or the bending and twisting characteristics of a spring produced from a wire, by applying stresses on the wire or bombarding the wire with metal shot.

JP-A 57 210 916 discloses a high strength steel wire for a spring which is said to have superior bending and twisting characteristics. According to JP-A 57 210 916 compressive residual stress is produced in the surface layer of the wire by a liquid honing or shot peening effect and further compressive residual stress is applied to the surface layer of the wire by means of a wire brushing device after a cold drawing stage.

From "Herstellung von Stahldraht", 1969, Part 1, pages 187, 225 and 257 to 260 it can be taken that, when drawing steel wire, tensile stresses in the outer portions of the wire and compressive stresses in the center of the wire or visa versa can be produced, depending on the reduction applied. When roll- straightening the wire asymmetries of the stresses can be eliminated under certain circumstances.

DE-C 747 761 describes a method of improving the durability of wire springs in which the wire surface is compressed before coiling the wire into spring. It may be assumed that the compression is done by rolling.

GB-A 531 017 discloses a method of increasing the strength of a steel or steel alloy wire and its resistance to fatigue by subjecting the wire, as a final operation in its manufacture, to a continuous bombardment with round metal shot or metal globules. In GB-A 531 017 it is also mentioned that it is already known to surface harden steel articles by subjecting them to bombardment by a stream of metal shot.

"Stahl und Eisen" Vol. 104 (1984) No. 14, pages 657 to 660 describes the plastic deformation of steel surfaces by rolling in order to improve the surface properties and the strength of the steel by means of various roll arrangements.

It is the object of the invention to provide a high tensile strength steel wire with excellent and increased ductility, and a method of producing such a wire.

This object is achieved by the steel wire and the method according to the claims 1 and 6, respectively. Optional features of the invention are mentioned in the dependent claims.

The invention is described in detail in connection with the drawings in which
Fig. 1 is an illustration of a typical method of working or deforming the surface of a steel wire by rolling;
Fig. 2 illustrates a typical rolling instrument in detail;
Figs. 3A, 4A and 4B are side and front views of rollers;
Fig. 5 is an illustration of a typical method of working or deforming the surface of a steel wire by shot peening;
Figs. 6 and 7 are typical illustrations of normal and abnormal ways by which a steel wire breaks in a torsion test, respectively; and
Fig. 8 shows a longitudinal crack appeared on a wire surface in a torsion test.

A steel wire of the present invention contains the following chemical components in amounts described below.

It contains 0.4 to 1.0% C, because, if the content thereof were less than 0.4%, the required strength is not attained, and with over 1.0% C, the ductility of the resulting steel wire is greatly decreased.

Si is added because it is capable of setting a solid solution hardening, and the amount employed is limited to 2.0% or less, since the ductility becomes decreased when over 2% Si is contained in a steel wire.

Mn is contained to assure hadenability and fix S as MnS, and the amount thereof is set at between 0.2 and 2.0%, since less than 0.2% Mn is not capable of sufficiently fixing S and the hardenability thereof does not increase with a content of over 2% Mn.

The less P and S the steel wire contains, the better is its quality in terms of improved ductility. Ductility is deteriorated conspicuously with over 0.02% of either, and the amont thereof is therefore limited to 0.02% or less.

N is contained in an amount of 0.01% or less, since with a content of over 0.01% N thereof a deterioration in the ductility is apparent.

The thus-composed steel wire of the present invention optionally contains, in addition to the ingredients described above, at least one ingredient selected from group (A) consisting of 0.05 to 3% of Cr, 0.01 to 1% of Mo, 0.01 to 1% of W, 0.05 to 3% of Cu, 0.1 to 5% of Ni and 0.1 to 5% of Co, and/or at least one ingredient selected from group (B) consisting of 0.001 to 0.1% of AI, 0.001 to 0.1% of Ti, '0.001 to 0.1% of Nb, 0.001 to 0.1% of V, 0.0003 to 0.05% of B, 0.001 to 0.1% of Mg and 0.001 to 0.1% of Ca.

Cr, Mo, W, Cu, Ni and Co are incorporated for the purpose of increasing the strength and corrosion resistance. They are not effective if added in amounts of less than 0.05%, 0.01%, 0.01%, 0.05%, 0.1% and 0.1%, respectively. The lower limit of the specified amounts thereof are therefore set at 0.05%, 0.01 %, 0.01 %, 0.05%, 0.1 % and 0.1 %, respectively.

Cr, Mo, W, Cu, Ni and Co are incorporated in amounts which are less than or equal to 3%, 1%, 1%, 3%, 5% and 5%, respectively. This is because when the content exceeds these amounts, the ductility of the steel wire is lowered, while the increase in strength and corrosion resistance is saturated. It is preferable for the total amount of these elements to be set at 7% or less from the viewpoint of good ductility.

Al, Ti, Nb, V, B, Mg and Ca are added in the steel wire for the purpose of increasing the ductility thereof by fixing N and S. Their effects are not apparent, however, if added in amounts which are less than 0.001%, 0.001%, 0.001%, 0.0003%, 0.001% and 0.001%, respectively. The amounts thereof are therefore set to be at least 0.001%, 0.001%, 0.001%, 0.0003%, 0.001% and 0.001%, respectively.

If, on the other hand, Al, Ti, Nb, V, B, Mg and Ca are added in amounts which are over 0.1%, 0.1%, 0.1%, 0.1%, 0.05%, 0.1% and 0.1%, respectively, the ductility of the steel wire is decreased due to the resulting nitride and sulfide of these elements, while their respective effects are saturated. The amounts thereof to be added are therefore set to be no more than 0.1 %, 0.1 %, 0.1 %, 0.1 %, 0.05%, 0.1 % and 0.1 %, respectively. The total amount of these elements is preferably set at 0.2% at most to ensure the quality in terms of ductility.

The steel wire of the present invention has a strength to of at least 130 kgf/mm², since, if the strength is less than 130 kgf/mm², the ductility does not increase even if there is a residual compression stress on the surface of the steel wire.

The steel wire according to the present invention has a residual compression stress of between (0.05 a + 23) and (0.35 α + 28) kgf/mm² on the surface thereof, depending on its strength α, for the reasons described below.

The ductility of steel wire is generally determined by tensile, torsion and bending tests, based on such results as the elongation and reduction of area observed in the tensile test, and the number of turns (torsion number) to fracture and the mode of that fracture observed in the torsion test.

Of all these measures of ductility, the mode of fracture in torsion test is deteriorated mostly when the strength of the steel wire is increased.

Figs. 6 and 7 illustrate typical ways in which a steel wire 2 fractures in torsion tests. Fig. 6 shows a normal mode of fracture in steel wire, while Fig. 7 illustrates an abnormal fracture with cracks 11. The abnormal type of fracture occurs more frequently as the strength of the steel wire 2 increases. It is caused by the occurence of a longitudinal crack 11 as shown in Fig. 8, in which a wire is twisted by cuck- ing with jig 12. It can therefore be considered that abnormal fracture means a deterioration in the ductility in the circumferential direction of the steel wire.

The fact that an increase in the strength of the steel wire decreases the ductility in the circumferential direction is most clearly related to the phenomena whereby the steel wire cracks often in the longitudinal direction during bending, before failure occurs, and whereby longitudinal cracks occur frequently during the bunching of the steel wire, before failure occurs. It is understood from the foregoing description that the manner in which fracture occurs in a torsion test is the most important criterion of the ductility of steel wire.

The present inventors have found that the ductility of steel wire in the circumferential direction can be effectively increased by providing its surface with a residual compression stress, and they have studied the appropriate range for the application of this residual compression stress. More specifically, the present inventors set themselves the goal of reducing the incidence of abnormal fracture to 10% or less in torsion tests, and investigated how the level of the surface residual compression stress and the occurrence of abnormal fracture are related, using steel wire having tensile strengths of 152 kgf/mm2, 235 kgf/mm2, 316 kgf/mm2 and 377 kgf/mm², respectively.

From the results obtained, it was concluded that it is essential for steel wires having tensile strengths of 152 kgf/mm², 235 kgf/mm², 316 kgf/mm² and 377 kgf/mm² to possess a residual compression stress of at least 29 kgf/mm^{z}, 36 kgf/mm², 38 kgf/mm² and 42 kgf/mm², respectively to 10% or less, on the basis of torsion tests which were conducted. Each of these residual compression stresses, when observed relative to the corresponding tensile strength α, was found experimentally to be equal to (0.05 α + 23) kgf/mm². If the incidence of abnormal fracture is reduced to 10% or less in such torsion tests, there is no problem related to the occurrence of longitudinal cracks during the practical processing of the steel wire. Thus, the lower limit of the residual compression stress to be applied to the surface of steel wire was set at (0.05 a + 23) kgf/mm². This value of course changes as the strength of the wire increases.

The higher the residual compression stress applied to the surface of the steel wire, the better its ductility in the circumferential direction. However, the residual tensile stress at the center of the steel wire increases in proportion to the residual compression stress on the surface, as is generally known, and cracks thereby occur in the center which lead to abnormal fracture in torsion tests. This determines the maximum allowable residual compression stress which can be applied to the surface. The present inventors have investigated how the occurrence of abnormal fracture due to cracks generated in the center of the steel wire is related to the level of residual compression stress which is applied, using four types of steel wires of the same strengths as those employed before.

From the results of these investigations, it was concluded that abnormal fractures begin to occur in steel wires which have tensile strengths of 152 kgf/mm², 235 kgf/mm², 316 kgf/mm2 and 377 kgf/mm2, respectively, when the residual compression stresses applied to the surfaces exceed 80 kgf/mm², 113 kgf/mm2, 136 kgf/mm2 and 160 kgf/mm², respectively. The residual compression stresses are proportional to the corresponding wire strengths α, and were found experimentally to be equal to (0.35 a + 28) kgf/mm2. The upper limit of the residual compression stress to be applied was thus determined to be (0.35 a + 28) kgf/mm2.

Subsequently, the present inventors made a quantitative study to clear the appropriate range of application of strain by means of surface deformation which is required to maintain the surface residual compression stress in the above-described range, and found that the strain should be limited to between 0.2 and 10% to do so. This is because, if the strain is less than 0.2%, residual compression stress within the above-described range cannot be applied on the surface. On the other hand, fine cracks appear on the surface of a steel wire and the ductility thereof tends to decrease when the strain exceeds 10%. Thus, the range of strain application by surface deformation is restricted to between 0.2 and 10%.

The residual compression stress of the above-described range is practically applied to the surface of a steel wire by deforming its surface such as to impart a strain of between 0.2 and 10% in the following manner.
Fig. 1 illustrates a typical method of applying surface residual compression stress by rolling. In the Figure, the steel wire 2 is unwound from an unwinding machine 6, is passed through a pinch roller 7, and is wound on a winding machine 8. The pinch roller 7 is adapted to supply a tension to the steel wire 2. The surface of the steel wire 2 is deformed by a rolling machine 3 located between the pinch roller 7 and the winding machine 8.
Fig. 2 shows the rolling machine jig 3 in detail. Strain is applied to the surface of the steel wire 2 by passing it between a plurality of spherical rollers 1 which are rotated by being rubbed against the passing steel wire. The amount of strain to be applied may be controlled by adjusting the rolling reduction of the rollers 1.

Rollers of a disk-shaped configuration as shown in Figs. 3A, 3B and 4A, 4B may also be employed. In such a case, it is necessary for the end of the rollers 20 and 21 to have a flat or convex shape. This is because the experiments confirmed that if the configuration thereof is concave, it is impossible to apply a surface residual compression stress at a level in the above-described range.

The rolling machine jig 3 may include more than one pair of rollers. This may be a more effective way of carrying out the present invention than employing just one pair of rollers.

The present invention may be carried out more effectively by transmitting the rotation of a motor 5 to the rolling machine 3 through a shaft 4 and rotating the rolling machine 3 about the steel wire 2. At this time, if the rollers employed are of a disk-like shape, the rollers are disposed at a certain angle relative to the steel wire 2.

Fig. 5 illustrates a typical method of applying a residual compression stress to the surface by shot peening a steel wire. A shot 9 may be blasted through a pipe 10 by means of compressed air or by rotating the jig 3 about the steel wire so as to deform the surface of the steel wire.

This surface deformation may be conducted immediately after the steel wire comes out of the dies in the wire drawing process or at any time before completion of the final product. If the surface of the steel wire is deformed after blueing or plating, however, it is preferable for the steel wire to be blued again at a temperature of 250_{°}C or less so as to improve the stress relaxation.

At this time, it is preferable for the difference in hardness between the core and surface of the steel wire to be set at 100 or less in vickers hardness. This is because if it exceeds 100, the steel wire may crack during rolling.

A steel wire of the present invention exhibits excellent characteristics in terms of fatigue, corrosion fatigue, delayed fracture, stress corrosion cracking or relaxation properties.

When employed in such products as ropes, steel wire reinforced tires and steel wire reinforced plastics, the steel wire of the present invention is capable of improving the durability or fatigue characteristics of these products.

The present invention will be described hereinunder by way of examples.

Table 1 lists the compositions, diameters, tensile strengths of the steel wires employed in the examples, the minimum values (0.05 a + 23) and the maximum values (0.35 a + 28) of residual compression stresses which can be applied to the surfaces of the steel wires which are determined in accordance with the present invention, the residual stresses existing on the surfaces of the steel wires employed in the examples, the results of tests for twisting, fatigue, corrosion fatigue, delayed fracture, and relaxation on these steel wires, and the results of a fatigue test conducted on products employing these steel wires.

The results of the tests listed in the table are expressed as follows.

The symbol + in the item for residual stress indicates that the residual stress is one of tension, while the symbol - means that the stress is one of compression.

Abnormal type fracture frequencies refer to occurrences of the abnormal type of fracture shown in Fig. 7 in the torsion tests conducted.

Fatigue limits indicate stresses at the fatigue limits observed in the rotary bending tests conducted.

Breakage ratios of cords in tires are those for cords employed in tires subjected to a load of 500 kg while running 100,000 km.

Relaxation rates show the residual shear strains observed in steel wires 96 hours after being subjected to torsional stress equivalent to 60% of the maximum torsional strength..

Delayed fracture hours refer to the hours to fracture of steel wires when subjected to a tensile stress of 80 kgf/mm² in a solution of 0.1 N hydrochloric acid.

Fatigue limits of plastic plates refer to the bending fatigue limits observed in plastic plates having a thickness of 1 mm and a width of 10 mm reinforced by 100 steel wires per 1 mm ². These are expressed by the ratio of the measured value to that of No. 31 sample.

Corrosion fatigue lives represent the number of rotations to fracture of steel wires when subjected to a load of 20 kgf/mm² in rotary bending fatigue tests conducted in a 3% NaCI solution.

Stress corrosion cracking hours represent the hours to fracture of steel wires when subjected to a tensile strength of 70 kgf/mm2 in a solution of 0.5% acetic acid + 5% NaCi.

Rope fatigue limits show the bending fatigue limits of ropes which conform to JIS No. 1. The rope made from the steel wire shown in example No. 47 of this invention was compared with one made from the steel wire of comparison example No. 48, and the fatigue limits of these ropes were expressed by the ratio of the measured value to that of No. 31 sample.

In Table 1, the test Nos. which are circled indicate examples of this invention. The others represent comparison examples.

Tests Nos. 1 and 2 use steel wires having diameters of 0.2 mm and the tensile strengths of 332 kgf/mm² and composed of the same chemical components. The steel wire of No. 1 had a residual compression stress of 112 kgf/mm² which was imparted by applying a strain of 1.2% by rolling, and showed an abnormal fracture ratio of 0 in the torsion test conducted. On the other hand, the steel wire of test No. 2 had a residual tensile stress of 61 kgf/mm², and showed an abnormal fracture rate of 100%. This shows that the steel wire of this invention is excellent in ductility. The steel wire of this invention also exhibited excellent characteristics in terms of corrosion fatigue properties as well as durability when employed in a tire.

Tests Nos. 3 and 4 employed steel wires respectively having diameters of 2.6 mm and 4.5 mm, tensile strengths of 168 kgf/mm² and 196 kgf/mm², and residual compression stresses of 50 kgf/mm² and 83 kgf/mm². Both showed an abnormal fracture ratio of 0, and were excellent in ductility. For both wires, the residual compression stresses were imparted by applying strains of 0.3% and 0.9%, respectively, by shot peening.

Tests Nos. 5, 6, 7 and 8 used steel wires having compositions and residual stresses outside the scope of the present invention. Hence, these showed high rates of abnormal fracture and poor ductility.

Nos. 9 and 10 represent the tests employing steel wires having diameters of 0.25 mm, tensile strengths of 286 kgf/mm², and the same composition. The steel wire of test No. 9 had a residual compression stress of 87 kgf/mm², and showed an abnormal fracture ratio of 5% in the torsion test conducted, while the steel wire of No. 10 had a residual tensile stress of 45 kgf/mm², and therefore showed an abnormal fracture ratio of 95%. From these tests, it is clear that the steel wire according to the present invention has excellent ductility. The residual compression stress was imparted to both steel wires by applying a strain of 6.2% by rolling.

Test No. 11 employed a steel wire having a diameter of 2.5 mm, a tensile strength of 205 kgf/mm² and a residual compression stress of 60 kgf/mm^{2.} The steel wire showed an abnormal fracture ratio of 0, which shows that the ductility thereof was excellent. The residual compression stress was imparted by applying a strain of 1.0% by shot peening.

Tests Nos. 12 and 13 represent examples of steel wires having diameters of 0.6 mm and tensile strengths of 256 kgf/mm² and which are composed of the same components. The steel wire of No. 12 had a residual compression stress of 65 kgf/mm², while that of No. 13 was 130 kgf/mm^{2.} The latter was imparted its residual compression stress by applying a rolling strain of 12%. The abnormal fracture ratio of No. 12 represented 5%, while that of No. 13 reached 70%. The steel wire of the present invention thus proved to be excellent in ductility. The residual compression stress was imparted to the steel wire of example No. 12 by applying a strain of 0.3% through rolling.

Tests Nos. 14 and 15 employed a steel wire and a galvanized steel wire, respectively, which had diameters of 4.5 mm and 3.2 mm, tensile strengths of 195 kgf/mm² and 179 kgf/mm² and residual compression stresses of 45 kgf/mm² and 41 kgf/mm², respectively. Both wires showed abnormal fracture ratio of 0, and proved to be excellent in ductility. The residual compression stresses were imparted to the steel wires of Nos. 14 and 15 by applying a strain of 2.0% through rolling and a strain of 0.5% through shot peening, respectively.

Tests Nos. 16 to 18 concern the steel wires having diameters of 8 mm and tensile strengths of 152 kgf/mm² which were composed of the same components. The steel wire of No. 16 had a residual compression stress of 41 kgf/mm², and showed an abnormal fracture ratio of 5%. Nos. 17 and 18 had a residual tensile stress of 25 kgf/mm^{z} and a residual compression stress of 18 kgf/mm2, respectively, and their abnormal fracture ratios respectively represented 60% and 45%. The steel wires of the present invention thus proved to have excellent ductility. The residual compression stresses were imparted to the steel wires of Nos. 16 and 18 by applying strains of 0.3% through shot peening and 0.8% through rolling, respectively. The steel wire of the present invention also exhibited excellent characteristics in relaxation and delayed fracture properties.

Tests Nos. 19 and 20 employed steel wires respectively having diameters of 1.2 mm and 3.6 mm, tensile strengths of 220 kgf/mm² and 184 kgf/mm² and residual compression stresses of 78 kgf/mm² and 50 kgf/mm². Both exhibited abnormal fracture ratios of 5% and 0%, respectively, and proved to be excellent in ductility. The residual compression stresses were imparted to both wires by applying strains of 0.5% and 3.2%, respectively, through rolling.

Nos. 21 to 27 represent comparison examples employing steel wires whose compositions and residual stresses are outside the scope of the present invention. Hence, both showed high abnormal fracture ratios and poor ductility.

Tests Nos. 28 and 29 used steel wires respectively having diameters of 2.0 mm and 0.8 mm, tensile strengths of 196 kgf/mm² and 258 kgf/mm², and residual compression stresses of 60 kgf/mm² and 72 kgf/mm². Abnormal fracture ratios for both wires showed 0 and 5%, respectively, and their ductilities proved to be excellent.

Tests Nos. 30 and 31 employed steel wires having diameters of 0.06 mm and tensile strengths of 408 kgf/mm2 which were composed of the same components. The steel wire of No. 30 had a residual compression stress of 76 kgf/mm², and showed an abnormal fracture ratio of 5%, while the steel wire of No. 31 had a residual tensile strength of 50 kgf/mm² and the abnormal fracture ratio thereof therefore represented 100%. Ductility of the steel wire in accordance with the present invention thus proved to be excellent. It also proved that the plastic plate reinforced by the steel wire according to the present invention had excellent fatigue property. The residual compression stress was imparted by applying a strain of 0.2% through rolling.

Test No. 32 concerns a steel wire having a diameter of 5.5 mm, a tensile strength of 185 kgf/mm² and a residual compression stress of 65 kgf/mm^{2.} The employed wire showed an abnormal fracture ratios of 0, and proved to be excellent in ductility.

Tests Nos. 33 and 34 represent examples employing steel wires having diameters of 3.2 mm and tensile strengths of 146 kgf/mm², which were composed of the same ingredients. The steel wire of No. 33 had a residual compression stress of 45 kgf/mm2, and showed an abnormal fracture ratio of 0. The steel wire of No. 34 had a residual compression stress as high as 93 kgf/mm² which was imparted thereto by applying a rolling strain of 15%, and hence showed an abnormal fracture ratio of 35%. This shows that the steel wire of the present invention was excellent in ductility.

Tests Nos. 35 and 36 used steel wires respectively having diameters of 3.2 mm and 0.3 mm, tensile strengths of 170 kgf/mm² and 238 kgf/mm² and residual compression stresses of 50 kgf/mm² and 69 kgf/mm². Abnormal fracture ratios for both steel wires represented 0 and 5%, respectively, and both proved to have excellent ductility. Residual compression stresses were imparted to the steel wires of Nos. 32, 33, 35 and 36 by applying strains of 0,8%, 0.2%, 2.0% and 1.2% through shot peening, respectively.

Tests Nos. 37 to 42 represent comparison examples employing steel wires having compositions and residual stresses outside the scope of the present invention. The abnormal fracture ratios of these steel wires were therefore high, and their ductilities were poor. An excessively high residual compression stress was imparted to the steel wire of No. 40 by applying a strain as high as 10.8% through rolling.

Tests Nos. 43 to 46 employed steel wires respectively having diameters of 2.0 mm, 3.6 mm, 1.2 mm and 0.35 mm, tensile strengths of 195 kgf/mm²,185 kgf/mm², 221 kgf/mm² and 260 kgf/mm², and residual compression stresses of 75 kgf/mm2, 50 kgf/mm2, 40 kgf/mm² and 80 kgf/mm². In all cases, the abnormal fracture ratios represented 0, and the ductilities proved to be excellent.

Tests Nos. 47 and 48 used steel wires having diameters of 3.6 mm, tensile strengths of 228 kgf/mm² and the same compositions. The steel wire of No. 47 had a residual compression stress of 63 kgf/mm2, showed an abnormal fracture ratio of 0 and proved to be excellent in ductility. The steel wire of No. 48, on the other hand, had a residual tensile stress of 30 kgf/mm², and the abnormal fracture ratio thereof represented 75%. This shows that its ductility was poor.

The steel wire of No. 47 proved also to be excellent in stress corrosion cracking property. The rope made of this steel wire showed excellent characteristics in fatigue properties.

The residual compression stresses were imparted to the steel wires of Nos. 43, 44, 45, 46 and 47 by applying rolling strains of 3.0%, 0.6%, 7.8%, 1.0% and 1.5%, respectively.

Tests Nos. 49 and 50 employed steel wires having diameters of 0.6 mm, tensile strengths of 290 kgf/mm2 and the same compositions. The steel wire of No. 49 had a residual compression stress of 86 kgf/mm², and showed an abnormal fracture ratio of 0, which represents excellent ductility. On the other hand, a residual tensile stress as high as 43 kgf/mm² was imparted to the steel wire of No. 50, and the abnormal fracture ratio thereof rose as high as 90%. It is clear that the steel wire of No. 50 had poor ductility. The steel wire of No. 49 also exhibited excellent characteristics in fatigue properties. The residual compression stress was imparted to the wire of No. 49 by applying a strain of 0.7% through shot peening.

Tests Nos. 51 to 55 represent comparison examples employing steel wires having compositions and residual stresses outside the scope of the present invention. The abnormal fracture ratios of these steel wires were therefore high with poor ductility. The steel wire of No. 54 was subjected to a strain as high as 11.6% by rolling, and had a large residual compression stress.

The difference in the hardnesses of the core and the surface of each steel wire according to the present invention represented a Vickers hardness of less than 100. The hardness difference in the case of the steel wires belonging to comparison examples Nos. 5, 26, 38 and 54, however, exceeded 100.

## Claims

1. A high tensile strength drawn steel wire having excellent ductility, comprising a steel containing 0.4 to 1.0% by weight of C, 2.0% or less by weight of Si, 0.2 to 2% by weight of Mn, 0.02% or less by weight of P, 0.02% or less by weight of S and 0.01% or less by weight of N, and optionally further containing: at least one ingredient selected from the group consisting of 0.05 to 3% by weight of Cr, 0.01 to 1% by weight of Mo, 0.01 to 1% by weight of W, 0.05 to 3% by weight of Cu, 0.1 to 5% by weight of Ni and 0.1 to 5% by weight of Co, and/or at least one ingredient selected from the group consisting of 0.001 to 0.1% by weight of Al, 0.001 to 0.1% by weight of Ti, 0.001 to 0.1% by weight of Nb, 0.001 to 0.1% by weight of V, 0.0003 to 0.05% by weight of B, 0.001 to 0.1% by weight of Mg, and 0.001 to 0.1% by weight of Ca, balance Fe and unavoidable impurities, wherein said steel has a strength σ of between (0.05 a + 23) and (0.35 α + 28) kgf/mm² on the surface thereof, depending on its strength «.

2. The steel wire of claim 1, wherein said steel is hot rolled and said hot rolled or heat treated steel is drawn to prepare a steel wire having said strength α, said steel wire being subjected to surface deformation so as to impart a strain of between 0.2 and 10% and thereby apply a said residual compression stress on its surface.

3. The steel wire of claim 2, wherein said surface deformation is done by rolling with spherical rollers.

4. The steel wire of claim 2, wherein said surface deformation is done by rolling with disk-like shaped rollers.

5. The steel wire of claim 2, wherein said surface deformation is done by shot peening.

6. A method of producing a high tensile strength drawn steel wire having excellent ductility, the steel composition of said drawn steel wire containing 0.4 to 1.0% by weight of C, 2.0% or less by weight of Si, 0.2 to 2% by weight of Mn, 0.02% or less by weight of P, 0.02% or less by weight of S and 0.01% or less by weight of N, and optionally further containing: at least one ingredient selected from the group consisting of 0.05 to 3% by weight of Cr, 0.01 to 1% by weight of Mo, 0.01 to 1% by weight of W, 0.05 to 3% by weight of Cu, 0.1 to 5% by weight of Ni and 0.1 to 5% by weight of Co, and/or at least one ingredient selected from the group consisting of 0.001 to 0.1% by weight of Al, 0.001 to 0.1% by weight of Ti, 0.001 to 0.1 % by weight of Nb, 0.001 to 0.1% by weight of V, 0.003 to 0.05% by weight of B, 0.001 to 0.1% by weight of Mg, and 0.001 to 0.1% by weight of Ca, balance Fe and unavoidable impurities, said method comprising the step of applying strain to the wire by means of surface deformation, said strain being limited to between 0.2 and 10% so that said steel has a strength σ of 130 kgf/mm² or more and a residual compression stress of between (0.05 a + 23) and (0.35 a + 28) kgf/mm² on the surface thereof, depending on its strength σ.

7. The method of claim 6, wherein said surface deformation is done by rolling with spherical rollers.

8. The method of claim 6, wherein said surface deformation is done by rolling with disk-like shaped rollers.

9. The method of claim 6, wherein said surface deformation is done by shot peening.

## Patentansprüche

1. Gezogener Stahldraht mit hoher Zugfestigkeit und ausgezeichneter Duktilität, welcher einen Stahl aufweist, der enthält: 0,4 bis 1,0 Gew.-% C, höchstens 2,0 Gew.-% Si, 0,2 bis 2,0 Gew.-% Mn, höchstens 0,02 Gew.-% P, höchstens 0,02 Gew.-% S und höchstens 0,01 Gew.-% N, und welcher ferner gegebenenfalls enthält: mindestens einen Bestandteil aus der Gruppe bestehend aus 0,05 bis 3 Gew.-% Cr, 0,01 bis 1 Gew.-% Mo, 0,01 bis 1 Gew.-% W, 0,05 bis 3 Gew.-% Cu, 0,1 bis 5 Gew.-% Ni und 0,1 bis 5 Gew.-% Co, und/oder mindestens einen Bestandteil aus der Gruppe bestehend aus 0,001 bis 0,1 Gew.-% Al, 0,001 bis 0,1 Gew.-% Ti, 0,001 bis 0,1 Gew.-% Nb, 0,001 bis 0,1 Gew.-% V, 0,003 bis 0,05 Gew.-% B, 0,001 bis 0,1 Gew.-% Mg und 0,001 bis 0,1 Gew.-% Ca, Rest Eisen und unvermeidbare Verunreinigungen, wobei der Stahl eine Festigkeit σ von mindestens 130 kgf/mm² und eine von seiner Festigkeit σ abhängige Restdruckspannung zwischen (0,05 a + 23) und (0,35 σ + 28) kgf/mm² an seiner Oberfläche aufweist

2. Stahldraht gemäß Anspruch 1, wobei der Stahl warmgewalzt und der warmgewalzte oder wärmebehandelte Stahl gezogen wird, um einen Stahldraht mit der besagten Stärke σ zu erzeugen, wobei der Stahldraht einer Oberflächendeformation unterzogen wird, um ihm eine Verformung von 0,2 bis 10% zu verleihen und dadurch die Restdruckspannung auf seine Oberfläche aufzubringen.

3. Stahldraht nach Anspruch 2, wobei die Oberflächendeformation durch Walzen mit sphärischen Walzen durchgeführt wird.

4. Stahldraht nach Anspruch 2, wobei die Oberflächendeformation durch Walzen mit scheibenartig geformten Walzen durchgeführt wird.

5. Stahldraht nach Anspruch 2, wobei die Oberflächendeformation durch Kugelstrahlen durchgeführt wird.

6. Verfahren zum Herstellen eines gezogenen Stahldrahts mit hoher Zugfestigkeit und ausgezeichneter Duktilität, wobei die Stahlzusammensetzung des gezogenen Stahldrahts aufweist: 0,4 bis 1,0 Gew.-% C, höchstens 2,0 Gew.-% Si, 0,2 bis 2 Gew.-% Mn, höchstens 0.02 Gew.-% P, höchstens 0,02 Gew.-% S und höchstens 0,01 Gew.-% N, und gegebenenfalls ferner enthält: mindestens einen Bestandteil aus der Gruppe bestehend aus 0,05 bis 3 Gew.-% Cr, 0,01 bis 1 Gew.-% Mo, 0,01 bis 1 Gew.-% W, 0,05 bis 3 Gew.-% Cu, 0,1 bis 5 Gew.-% Ni und 0,1 bis 5 Gew.-% Co, und/oder mindestens einen Bestandteil aus der Gruppe bestehend aus 0,001 bis 0,1 Gew.-% Al, 0,001 bis 0,1 Gew.-% Ti, 0,001 bis 0,1 Gew.-% Nb, 0,001 bis 0,1 Gew.-% V, 0,0003 bis 0,05 Gew.-% B, 0,001 bis 0,1 Gew.-% Mg, und 0,001 bis 0,1 Gew.-% Ca, Rest Eisen und unvermeidbare Verunreinigungen, wobei das Verfahren den Verfahrensschritt aufweist, daß auf den Draht mittels Oberflächendeformation eine Verformung ausgeübt wird, wobei die Verformung auf 0,2 bis 10% begrenzt ist, so daß der Stahl eine Festigkeit a von mindestens 130 kgf/mm² und eine von der Festigkeit σ abhängige Restdruckspannung zwischen (0,05 σ + 23) und (0,35 a + 28) kgf/mm² auf seiner Oberfläche aufweist

7. Verfahren nach Anspruch 6, wobei die Oberflächendeformation durch Walzen mit sphärischen Walzen durchgeführt wird.

8. Verfahren nach Anspruch 6, wobei die Oberflächendeformation durch Walzen mit scheibenartig geformten Walzen durchgeführt wird.

9. Verfahren nach Anspruch 6, wobei die Obertlächendeformation durch Kugelstrahlen durchgeführt wird.

## Revendications

1. Fil d'acier tréfilé à haute résistance à la traction présentant une excellente ductilité, comprenant de l'acier contenant 0,4 à 1,0% en poids de C, 2,0% ou moins en poids de Si, 02 à 2% en poids de Mn, 0,02% en poids ou moins de P, 0,02% en poids ou moins de S et 0,01% en poids ou moins de N, et contenant facultativement en outre: au moins un ingrédient sélectionné dans le groupe constitué par 0,05 à 3% en poids de W, 0,05 à 3% en poids de Cu, 0,1 à 5% en poids de Ni et 0,1 à 5% en poids de Co, et/ou au moins un ingrédient sélectionné dans le groupe constitué par 0,001 à 0,1% en poids de AI, 0,001 à 0,1% en poids de Ti, 0,001 à 0,1% en poids de Nb, 0,001 à 0,1 % en poids de V, 0,003 à 0,05% en poids de B, 0,001 à 0,1 % en poids de Mg et 0,001 à 0,1% en poids de Ca, le complément étant constitué par du Fe et les impuretés inévitables, caractérisé en ce que ledit acier présente une résistance a de 130 kgf/mm2 ou davantage et une contrainte de compression résiduelle comprise entre (0,05 α + 23) et (0,35 α + 28) kgf/mm² sur sa surface, en fonction de sa résistance α.

2. Fil d'acier selon la revendication 1, caractérisé en ce que cet acier est laminé à chaud et en ce que ledit acier laminé à chaud ou traité thermiquement est tréfilé afin de préparer un fil d'acier présentant ladite résistance α, ce fil d'acier étant soumis à une déformation de surface de manière à lui conférer une contrainte comprise entre 0,2 et 10% et a ainsi appliquer sur sa surface ladite contrainte de compression résiduelle.

3. Fil d'acier selon la revendication 2, caractérisé en ce que ladite déformation de surface est effectuée par laminage au moyen de laminoirs sphériques.

4. Fil d'acier selon la revendication 2, caractérisé en ce que ladite déformation de surface est effectuée au moyen de laminoirs en forme de disque.

5. Fil d'acier selon la revendication 2, caractérisé en ce que ladite déformation de surface est effectuée par grenaillage.

6. Procédé de production d'un fil d'acier tréfilé à haute résistance à la traction présentant une excellente ductilité, la composition de l'acier dudit fil d'acier tréfilé étant de 0,4 à 1,0% en poids de C, 2,0% en poids ou moins de Si, 0,2 à 2% en poids de Mn, 0,02% en poids ou moins de P, 0,02% en poids ou moins de S et 0,01% en poids ou moins de N, et contenant facultativement en outre: au moins un ingrédient sélectionné dans le groupe constitué par 0,05 à 3% en poids de Cr, 0,01 à 1% en poids de Mo, 0,01 à 1% en poids de W, 0,05 à 3% en poids de Cu, 0,1 à 5% en poids de Ni et 0,1 à 5% en poids de Co, et/ou au moins un ingrédient sélectionné dans le groupe constitué par 0,001 à 0,1% en poids de AI, 0,001 à 0,1% en poids de Ti, 0,001 à 0,1 % en poids de Nb, 0,001 à 0,1 % en poids de V, 0,0003 à 0,05% en poids de B, 0,001 à 0,1% en poids de Mg, et 0,001 à 0,1% en poids de Ca, le complément étant constitué par du Fe et les impuretés inévitables, ce procédé comprenant l'étape consistant à appliquer une contrainte au fil par une déformation de surface, ladite contrainte étant limitée à une valeur comprise entre 0,2 et 10% de manière à ce que ledit acier ait une résistance a de 130 kgf/mm² ou davantage et une contrainte de compression résiduelle comprise entre (0,05 a + 23) et (0,35 a + 28) kgf/mm² sur sa surface, en fonction de sa résistance a.

7. Procédé selon la revendication 6, caractérisé en ce que ladite déformation de surface est effectuée par laminage au moyen de laminoirs sphériques.

8. Procédé selon la revendication 6, caractérisé en ce que ladite déformation de surface est effectuée au moyen de laminoirs en forme de disque.

9. Procédé selon la revendication 6, caractérisé en ce que ladite déformation de surface est effectuée par grenaillage.
